

## UNITED STATES PATENT OFFICE

HEINRICH WAGNER, OF FRANKFORT-ON-THE-MAIN, GERMANY, ASSIGNOR TO I. G. FARBENINDUSTRIE AKTIENGESELLSCHAFT, OF FRANKFORT-ON-THE-MAIN, GERMANY, A CORPORATION OF GERMANY

## PROCESS FOR PREPARING HAIR TO BE WORKED INTO FELT

No Drawing. Application filed March 26, 1926, Serial No. 97,779, and in Germany April 9, 1925.

It is known that it is the practice in the manufacture of hats from hair to impregnate the unprepared rabbit and hare skins with solutions of nitrate of mercury, in order to 5 increase the felting property of the hair. The said mercury solutions are, however, extremely poisonous and in applying them with brushes the workmen handling them are spattered therewith.

10 Now, several attempts have already been made to find a substitute for the said poisonous mercury solution and there were proposed for this purpose solutions of iron, antimony, potassium, sodium, tin or the like in 15 nitric acid or sulfuric acid. From hair impregnated with these salts it was, indeed, possible to produce a felt, which, however, was not sufficiently firm and compact.

I have now found that an excellent felt 20 can be obtained by treating the skins with solutions of metallic salts, such as bismuth nitrate, zinc nitrate and aluminum nitrate, to which have been added such bodies as are adapted for use as wetting agents generally.

25 Among the bodies in question the organic sulfonic acids of higher molecular weight, particularly the sulfonic acids of aryl-, aralkyl- or alkyl-naphthalenes, have proved to be very useful for the purpose in question.

30 These latter sulfonic acid compounds may be designated as sulfonic acids of organic compounds having the general formula R—X, wherein R represents a naphthalene residue and X represents one of the groups alkyl, 35 aryl and aralkyl.

The following examples serve to illustrate my invention:

1. 500 grams of bismuth nitrate are treated with 1000 c.c. of concentrated nitric acid of 40° Bé. and the liquor is made up with water of ordinary temperature to 10 litres. To this solution are added 100 grams of benzylnaphthalenesulfonic acid, the latter being dissolved by stirring in the cold. The skins are 45 then brushed over with the said composition in the usual manner and dried.

2. 500 grams of zinc nitrate and 100 grams of zinc chloride are treated with 1100 c.c. of nitric acid of 40° Bé. and made up with water 50 to 10 litres. To this solution are added 150

grams of benzylnaphthalenesulfonic acid. The skins are brushed over in the usual manner with this composition and dried.

3. 500 grams of aluminum nitrate are treated with 500 c.c. of concentrated nitric acid of 40° Bé. and the liquor is made up to 5 litres; there are then added thereto 100 grams of sodium alkylnaphthylsulfonate. When the last mentioned product has dissolved, the skins are brushed over with the 60 composition in the usual manner and dried.

4. 500 grams of bismuth nitrate are treated with 1100 c.c. of concentrated nitric acid and the liquor is made up with water of ordinary 65 temperature to 4 litres. To this solution is added a solution of 10 grams of sodium nitrite in 100 cc. of water and the whole is made up to 5 litres. To the liquor are added 100 grams of benzylnaphthalene sulfonic acid and the skins are brushed over with the 70 composition in the usual manner.

## I claim:

1. In processes for the preparation of hair to be worked into felt, the step which consists in treating the hair to be felted with a 75 solution comprising bismuth nitrate and a sulfonic acid of a naphthalene compound.

2. In processes for the preparation of hair to be worked into felt, the step which consists in treating the hair to be felted with a solution comprising bismuth nitrate and a sulfonic acid of an organic compound having the general formula: R—X wherein R represents a naphthalene residue and X represents one of the groups alkyl, 80 aryl and 85 aralkyl.

3. As a new composition of matter, a preparation to be used in working hair into felt containing bismuth nitrate and a sulfonic acid of a naphthalene residue. 90

4. As a new composition of matter, a preparation to be used in working hair into felt containing bismuth nitrate and a sulfonic acid of an organic compound having the general formula: R—X wherein R represents a naphthalene residue and X represents one of the groups alkyl, aryl and aralkyl. 95

5. In processes for the preparation of hair to be worked into felt, the step which con- 100

sists in treating the hair to be felted with a solution of a compound of the following formula: Y.(NO<sub>3</sub>)<sub>3</sub>, wherein Y stands for aluminum or bismuth, said solution containing also a sulfonic acid of a naphthalene compound.

6. In processes for the preparation of hair to be worked into felt, the step which consists in treating the hair to be felted with a 10 solution of a compound of the following formula: Y.(NO<sub>3</sub>)<sub>3</sub>, wherein Y stands for aluminum or bismuth, said solution containing also a sulfonic acid of an organic compound having the general formula: R—X 15 wherein R represents a naphthalene residue and X represents one of the groups alkyl, aryl and aralkyl.

7. As a new composition of matter, a preparation to be used in working hair into felt containing a compound having the following formula: Y.(NO<sub>3</sub>)<sub>3</sub>, wherein Y stands for aluminum or bismuth, and a sulfonic acid of a naphthalene residue.

8. As a new composition of matter, a preparation to be used in working hair into felt containing a compound having the following formula: Y.(NO<sub>3</sub>)<sub>3</sub>, wherein Y stands for aluminum or bismuth, and a sulfonic acid of an organic compound having the general 30 formula: R—X wherein R represents a naphthalene residue and X represents one of the groups alkyl, aryl and aralkyl.

In testimony whereof, I affix my signature.

Dr. HEINRICH WAGNER.

35

40

45

50

55

60

65